# EUROPEAN PATENT SPECIFICATION

(11) **EP 0 689 480 B1**
(45) Date of publication and mention of the grant of the patent: **07.10.1998**
(21) Application number: 94910938.3
(22) Date of filing: 14.03.1994
(51) Int. Cl.: B05D 1/36, B05D 7/00

(54) **TWO STAGE POWDER APPLICATION METHOD**
ZWEISTUFIGES PULVERBESCHICHTUNGSVERFAHREN
PROCEDE D'APPLICATION DE POUDRE EN DEUX ETAPES

(30) Priority: 15.03.1993 JP 81440/93
(43) Date of publication of application: 03.01.1996
(73) Proprietor: NORDSON CORPORATION, Westlake Ohio 44145-1148 (US)
(72) Inventor: MATSUNAGA, Masafumi, Shinagawa-ku, Tokyo (JP)
(74) Representative: Findlay, Alice Rosemary
(86) International application number: US9402743
(87) International publication number: WO9421385

(56) References cited:
- EP-A- 0 523 761
- US-A- 3 348 995

## Description

### Field of the Invention

This invention relates to an improved method for powder coating.

### Background of the Invention

In many powder coating applications, the average particle diameter applied to the surface to be coated varies depending on the thickness of the coating. For instance, if a relatively thick coating is desired, particles having a thick diameter are used. If a relatively thin coating is desired, particles having a thin diameter are used.

However, with large sized particles, the applied coating or film does not always appear level and smooth, even if heating is used to coalesce the particles after contact on the surface. This poor leveling of large particles is particularly acute when the coating material is a thermosetting polymer. In some cases, the coating looks uneven, like the external surface of a lemon, an effect sometimes referred to in the industry as the "orange peel" phenomenon.

In contradistinction, leveling is more easily achieved with smaller sized particles. However, per particle, the ratio of surface area to weight becomes high, and bulk density drops. When the particles are applied by spraying, the effect of air resistance makes it difficult to maintain a straight flight path for long distances. The ability to maintain a straight flight path is referred to as linearity. For coating objects with hollow or recessed portions, penetration of the small powder particles to these surfaces is poor. This poor coverage necessitates an increase in powder ejection air pressure. However, this increased ejection air pressure results in increased flow volume, so that while this additional air pressure carries the particles farther it tends also to carry particles away from the surface when the transport air rebounds away from the surface.

Additionally, powder having a relatively small or fine particle size has a high manufacturing cost. Thus, despite its well known coating qualities, the industry has generally not used powders of relatively small size particles.

US-A-3348995 discloses a method of coating metal surfaces with polyethylene in which a thin first layer of high density polyethylene powder is applied as a primer and a thick second layer of low density polyethylene powder or of low density polyethylene sheet is applied on top of the first layer, so as to provide a strongly adherent protective coating of polyethylene.

It is an objective of this invention to improve the leveling and the aesthetic appearance of a powder coating applied to a surface, without compromising the delivery of the powder particles to the surface being coated or the adhesion of particles to the surface.

### Summary of the Invention

The invention relates to a method for powder coating a surface by
applying to the surface, during a first coating stage, powder particles having a first average diameter; the invention being characterised by the step of
applying to the surface, in a second coating stage, powder particles having a second average diameter smaller than the first average diameter, thereby to form a coating on the surface comprising particles applied during the first and second stages.

The present invention achieves the above-stated objectives by a two step particle application method which involves initially applying large size particles to a coating surface, followed by applying small particles to the surface. The average particle diameter for the powder applied during the first stage (Stage A) is 15 to 120 microns, and the average particle diameter for the powder applied during the second stage (Stage B) is 0.1 to 15 microns.

Preferably during both stages, the particles are applied by spraying. The larger sized particles applied during the first stage may be temporarily heated to cause partial melting and increased adherence. Subsequently, when the second stage particles are applied, heat may again be used to melt the applied powder particles. Stages A and B may be repeated as necessary, to achieve the desired coating thickness.

One advantage that results from this two stage powder application method is increased adhesion efficiency. Also, by initially applying the larger sized particles, the desired film thickness can be achieved, while subsequent application of the smaller sized particles improves overall leveling and surface appearance.

These and other features of the invention will be more readily understood in view of the following detailed description and the drawings.

### Brief Description of the Drawings

Fig. 1 is a cross-sectional view which schematically shows a powder coating achieved with the two stage powder application method of this invention, wherein the coated surface is flat.

Fig. 2 is a cross-sectional view, similar to Fig. 1, which schematically shows a powder coating achieved with the two stage powder coating method of this invention, wherein the coated surface has a recess.

Fig. 3 is a cross-sectional view, similar to Figs. 1 and 2 wherein the powder particles applied during the first stage are heated to achieve melting on the surface before the second stage of finer particles is applied.

### Detailed Description of the Preferred Embodiments

Fig. 1 depicts a surface 11 to be coated, and in this case the surface 11 is flat. The two stage powder application method of this invention involves initially applying to the surface 11 a powder 12 having a relatively large particle diameter. Preferably, the powder 12 has an average particle diameter in the range of about 15 to 120 microns. Subsequently, a powder 13 having a relatively small particle diameter is applied. Preferably, the powder 13 has an average particle diameter in the range of about 0.1 to 15 microns. Thus, the large particles 12 are applied during a first stage, while the smaller particles 13 are applied during a second stage. Preferably, the powder applied during the first and second stages are applied by spraying.

Because of the large particle diameter used in the first stage, the desired film thickness can be achieved. Subsequent application of the small particles 13 improves overall leveling and surface finish of the coating on the surface 11.

Fig. 2 illustrates another advantage of this two stage powder application method, an advantage which relates particularly to coating objects or articles which have an external surface with one or more hollow or recessed narrow portions, such as steel tools. Coating of objects such as this increases their resistance to rust. These objects usually also have one or more external surface sites which are more noticeable to consumers and thereby must have a favorable aesthetic appearance. A favorable appearance of this type generally requires coating with relatively small diameter particles. The two stage powder application method of this invention achieves both of these objectives, uniform coating of recessed narrow portions and an aesthetically pleasing coating on the external surface sites which are most noticeable to the consumer.

More particularly, Fig. 2 illustrates a portion of the surface 11 which has a recess 15 formed therein. Again, the coating on the surface 11 comprises an initial application of relatively large particles 12 followed by an application of small particles 13. The relatively large particles 12 used in the first stage of this method assure uniform coating within the recess 15, since the larger particles can penetrate into the recess to be deposited thereon, while the relatively small particles 13 level the overall coating of the entire surface 11 and further assure an aesthetically pleasing coating at the most noticeable sites.

One advantage of this method of powder coating is that in some applications where the coated object is subsequently processed, as in the bending of steel plates, cracks may occur in the coated film during this subsequent processing. However, with the two layers of coating applied according to this method, the bottom layer of large particles is relatively thick and has good workability and adhesive properties, while the top layer of small particles is formed of powder made of materials which are tough and have desired properties, such as chemical and/or weather resistance.

Another advantage of this invention relates to achieving a matted tone, a suede tone or a hammer tone coating for an article. These are design properties which have recently become popular in the market. By using, during the second stage, particles composed of urethane, polystyrene or glass beads which may be colored, it is easy to achieve a film with a matted or suede tone. Also, by using second stage particles which have a resin with poor compatibility with respect to the bottom layer, a hammer tone film can be achieved.

In the application of large particle diameter powders, and particularly those with a high molecular weight, it is difficult to achieve good levelling during heating and melting as noted above. The air present in the interstices between particles impairs levelling, and if the coated surface is too rapidly melted, the air surrounding the particles produces air bubbles. To solve these problems, this two stage powder application method involves temporarily heating the large size particles to melt them and subsequently applying the small size particles to cover the voids or pinholes in areas where the coating is thin or packed by air bubbles. This makes it possible to obtain a high quality film with no pinholes or voids and to achieve favorable levelling. The appearance of such a film is shown in Fig. 3, where reference numeral 16 designates the initially applied large particle diameter powder which is in a molten state due to temporary heating.

The invention contemplates the use of various types of powder. It is preferable to use an organic powder during the first stage, due to better adhesive properties. However, a mixture of inorganic and organic powders or a powder in which an organic powder is surrounded by organic capsules may also be used. This invention results in a high performance powder coating with relatively low costs, particularly when using powders such as fluorine and polyamide which are relatively expensive. Additionally, with a powder made of thermosetting material, due to differences in the catalyst, the hardener or the functional group used, compatibility may be poor and/or a phenomenon referred to as "crawling" may occur. Therefore, it is preferable to use powders composed of the same resin during Stage A and Stage B.

During powder coating, the phenomenon of levelling depends to a large extent on the surface tension during the melting of the powder materials. It has been found that a surface tension of 40 dyne/cm is preferred during melting of the powder. To maximize cost savings and productivity, it is desirable to use relatively large amounts of the large particle diameter powder and to increase the amount used during Stage A of particle application, since this powder is relatively inexpensive compared to the fine powder.

Also, by applying successive layers of powder having a large particle diameter and composed of a resin having a functional group and a small particle diameter powder composed of a hardener, the overall performance of the applied film can be improved. For example, this can be achieved by repeated application in overlapping layers or dispersion application of large diameter particles comprising a mixture of polyester and an isocyanate functional group and small diameter particles in which block isocyanate is encapsulated, followed by heating and melting or cross linking.

For each of these variations of the invention, this two stage powder application method produces a film or coating with favorable levelling, excellent aesthetic appearance, good linearity of the powder during application, good adhesion efficiency and high product quality.

While several preferred embodiments of the invention have been shown and described, it is to be understood that variations in these modifications may be made without departing from the scope of the invention. Accordingly, applicant wishes only to be bound by the claims appended hereto.

## Claims

1. A method for powder coating a surface (11) by
applying to the surface (11), during a first coating stage, powder particles (12) having a first average diameter; characterised by the step of
applying to the surface (11), in a second coating stage, powder particles (13) having a second average diameter smaller than the first average diameter, thereby to form a coating on the surface (11) comprising particles (12,13) applied
during the first and second stages.

2. The method of claim 1 wherein the first average diameter is in the range of about 15 to 120 microns and the second average diameter is in the range of about 0.1 and 15 microns.

3. The method of claim 1 and further comprising the steps of:
prior to the second coating stage, heating the powder particles (12) applied during the first coating stage to cause melting thereof, and subsequent to the second coating stage, heating all of the powder particles (12,13) to cause the particles applied during the first and second stages to melt and subsequently harden to form a coating.

4. The method of claim 1 wherein the first and second stage powders each have the same resin as a main component.

5. The method of claim 1 and further comprising repeating the steps to achieve a coating having a desired thickness.

6. The method of claim 1 wherein the particles are applied in both stages by spraying.

## Patentansprüche

1. Verfahren zum Pulverbeschichten einer Oberfläche (11) durch
Aufbringen von Pulverpartikeln (12) mit einem ersten mittleren Durchmesser auf die Oberfläche (11) in einer ersten Beschichtungsstufe; gekennzeichnet durch den Schritt des
Aufbringens von Pulverpartikeln (13) mit einem zweiten mittleren Durchmesser, der kleiner ist als der erste mittlere Durchmesser, auf die Oberfläche (11) in einer zweiten Beschichtungsstufe, wodurch eine Beschichtung auf der Oberfläche (11) gebildet wird, die aus während der ersten und zweiten Stufe aufgebrachten Partikeln (12, 13) besteht.

2. Verfahren nach Anspruch 1, bei dem der erste mittlere Durchmesser im Bereich von ungefähr 15 bis 120 µm und der zweite mittlere Durchmesser im Bereich von ungefähr 0,1 und 15 µm liegt.

3. Verfahren nach Anspruch 1, das außerdem die Schritte umfaßt:
Erwärmen der während der ersten Beschichtungsstufe aufgebrachten Pulverpartikel (12) vor der zweiten Beschichtungsstufe, um ihr Schmelzen zu bewirken, und auf die zweite Beschichtungsstufe folgend, Erwärmen aller Pulverpartikel (12, 13), um das Schmelzen der während der ersten und zweiten Stufe aufgebrachten Partikel zu bewirken, und nachfolgendes Aushärten zum Bilden einer Beschichtung.

4. Verfahren nach Anspruch 1, bei dem die Pulver der ersten und zweiten Stufe jeweils das gleiche Harz als einen Hauptbestandteil haben.

5. Verfahren nach Anspruch 1, und außerdem umfassend das Wiederholen der Schritte zum Erreichen einer Beschichtung mit einer gewünschten Dicke.

6. Verfahren nach Anspruch 1, bei dem die Partikel in beiden Stufen durch Spritzen aufgebracht werden.

## Revendications

1. Procédé de revêtement par poudre d'une surface (11) en
appliquant à la surface (11), pendant une première étape du procédé de revêtement, des particules de poudre (12) ayant un premier diamètre moyen,
caractérisée par l'étape consistant à :
appliquer à la surface (11), dans une deuxième étape du procédé de revêtement, des particules de poudre (13) ayant un deuxième diamètre moyen plus petit que le premier diamètre moyen, pour former ainsi un revêtement sur la surface (11) comprenant les particules (12, 13) appliquées durant les première et deuxième étapes.

2. Procédé selon la revendication 1, dans lequel le premier diamètre moyen est compris entre environ 15 et 120 microns et le deuxième diamètre moyen est compris entre environ 0,1 et 15 microns.

3. Procédé selon la revendication 1 et comprenant de plus les étapes consistant à :
avant la deuxième étape de revêtement, chauffer les particules de poudre (12) appliquée pendant la première étape de revêtement pour provoquer leur fusion et, après la deuxième étape de revêtement, chauffer toutes les particules de poudre (12, 13) pour conduire les particules appliquées pendant les première et deuxième étapes à fondre et durcir ensuite pour former un revêtement.

4. Procédé selon la revendication 1, dans lequel les poudres du premier et du deuxième étape ont chacune la même résine comme composant principal.

5. Procédé selon la revendication 1 et comprenant de plus le fait de répéter les étapes précédentes pour obtenir un revêtement ayant une épaisseur désirée.

6. Procédé selon la revendication 1, dans lequel les particules sont appliquées aux deux étapes par pulvérisation.
